

## UNITED STATES PATENT OFFICE

2,193,574

## PROCESS FOR THE PRODUCTION OF COLORED IMAGES BY PHOTOGRAPHY

Henricus Jacobus Charles Tendeloo, Wageningen, Netherlands, assignor to Shell Development Company, San Francisco, Calif., a corporation of Delaware

No Drawing. Application October 11, 1937, Serial No. 168,436. In the Netherlands October 21, 1936

15 Claims. (Cl. 95—7)

The present invention relates to a process for the production of colored images by photography, said colored images being produced in the film and in other light-sensitive layers, such as those on printing papers.

The introduction of sound and color into photography can be considered as very desirable improvements in the photographic art. Of these improvements the use of sound in conjunction with photography has been well developed while the introduction of color has been confined to a large extent to amateur use. Of the subtractive color processes developed, mention should be made of the Technicolor, Gaspar, Kodachrome and Agfa processes. These processes constitute technically improved processes based upon old ideas and have in general the disadvantage of requiring manifold and exacting processing and complicated and expensive methods of copying.

Since the ease of copying the films is of such paramount importance in the motion picture industry most of the above mentioned processes have not found extensive use in this field.

According to the present invention use is made of a light-sensitive compound which upon exposure to light of the proper wave length and if desirable development, liberates a fragment, ion or radical which remains to yield an image which corresponds in color to the natural color of the photographed object.

It is known that certain light-sensitive compounds upon being exposed to light of the proper wave length and to such development as may be desirable, break up, decompose, ionize or in some manner become separable into simpler materials. Thus, for example, the image of the ordinary black and white photograph is ascribed to metallic silver.

I have found that there are compounds which break down upon exposure into two fragments, one of which is colored or becomes colored after developing and the other of which may be selectively removed by suitable solvents. I also found that many of these colored fragments behave quite differently than the original unexposed compounds, thus allowing the selective removal of any unexposed compounds. Likewise, I have found that by the proper choice of radicals it is possible to produce colored images of almost any color by photography using these fragments to produce the colored images. Further, I have found that it is not essential that the fragment be colored per se, but that it is likewise possible to use such compounds as upon exposure and if desired development, yield uncolored fragments

which upon a simple treatment yield a stable colored image.

An example of a compound to be used in this manner is a metal salt of an oxamic acid, such as Ag, Cr, Hg, or Fe salt of o-nitro oxanilic acid. After exposure and development o-nitro aniline is formed, which is yellow. The metal liberated on exposure and the non-exposed salt are removed by a suitable bath, e. g. a KCN bath when Ag has been used as metal.

According to the present invention, any, preferably organic, dye compound which is light-sensitive and which after exposure and such development and fixation as the case may require leaves in the emulsion layer a colored material or a material capable of yielding a color upon a simple treatment, may be used. It is also possible to use a light-sensitive salt, which on exposure and such development as may be desired, decomposes into a fragment which is insoluble in the baths to be used and possesses per se, or upon a simple subsequent treatment, the desired color and a readily removable residue.

It is essential that the color-forming material liberated upon exposure to light and development be less soluble than the original unexposed compound, thus allowing the selective removal of any unexposed compound by solution.

An advantage of the present invention is that it is not restricted specifically to the use of salts of silver, mercury, chromium or iron, but that the light-sensitive hydrogen compounds and alkaline salts of the dye molecules can be used, since it is not the metal but essentially the dye base itself which is left in the emulsion layer. Thus the salts of Na, K, NH<sub>4</sub>, Cs, Rb, etc., may be used.

One suitable group of light-sensitive compounds is that of basic-acting dyes coupled with a polybasic acid, such as oxalic acid, and derivatives thereof.

The basic-acting dye can be coupled with the oxalic acid by means of a NH<sub>2</sub> group of the dye, whereby the oxalic acid derivatives of the general formula R<sub>1</sub>NR<sub>2</sub>CO.CO<sub>2</sub>X and homologues thereof are obtained, in which



contains the dye-carrying substance, and R<sub>1</sub> represents an organic dye-carrying radical, R<sub>2</sub> represents hydrogen or an organic radical and X represents a light-sensitive cation. The acids may be prepared, for example, by causing the

dye-carrying compound  $R_1R_2NH$  to act on ethyl oxalate. After saponification of the ethyl ester obtained, the acid



is formed. When  $R_2$  represents hydrogen, the acid  $R_1NH.CO.COONa$  is formed.

10 Thus, for example, the salts,



30 and the oxamine derivative of



may be advantageously used.

40 A basic-acting dye containing an OH-group can also be coupled with the polybasic acid by means of the OH-group, an ester being then formed of the general formula



in which  $B-OH$  represents the dye-carrying substance and  $X$  a light-sensitive cation. The reaction is then as follows:



in which  $B-OH$  is the basic-acting, OH-containing dye.

55 The emulsions may be sensitized to light of given wave lengths by the usual known methods. Different degrees of light sensitivity may also be attained by the use of isomeric compounds.

60 The unexposed light sensitive compound may be either colored or non-colored. If it is colored, this color should be taken into account in connection with sensitizing for a given light, since this color also absorbs part of the light. It is sometimes possible to use the sensitizer itself as a dye-carrying substance.

65 The image obtained may be improved by intensification or reduction by using special baths suitable for the particular dye-base.

70 In order to produce multicolored images, I prefer to apply the emulsions, each sensitized to a particular colored light, in layers on a suitable emulsion-carrier. In such cases where the sensitizing agents in two adjacent emulsion layers react to their mutual detriment, it is possible to eliminate this undesirable reaction by using as

75 a separator a layer of gelatin or other suitable

material. This separator-layer may contain a removable dye if desired, in which case it acts as a color filter. In some cases it is possible to mix the emulsions, each sensitive to a particular color, in which case the mixture may be applied to a suitable carrier and ripened.

As illustrative of a suitable manner in which my invention may be applied, I offer the following examples, which, it is to be understood, are not to be considered as limiting the scope of the invention as regards kind or proportions of materials used nor mode of execution:

*Example 1*

To one volume of an aqueous 8% gelatine solution at about 30° C. there was added one volume of a 1% solution of an oxamine derivative of mononitro benzidine, viz.



20

25 in water to which a small amount of  $NH_4OH$  had been added to aid the solution. To this was added 0.1 volume of a 0.01% thiosinamine solution in water and the whole thoroughly mixed. To this solution there was added, during intensive stirring a little more than the equivalent amount of  $\frac{1}{2}N$   $AgNO_3$  solution (in all about 0.075 volume of  $AgNO_3$  solution). The emulsion was poured over a suitable carrier and dried. The film thus prepared was exposed and then treated in a bath consisting of a 3% ammonium persulfate solution to which there had been added a few drops of a 3%  $KCN$  solution. The exposed portion remained behind as a red color.

*Example 2*

A light-sensitive silver salt of 6,6'-di-nitro-ortho-tolidine-dioxamic acid was obtained in the following manner: 1 milli-equivalent of the above oxamic acid was dissolved in 100  $cm^3$  water, in which 1 milli-equivalent  $NH_4OH$  was present. This solution was then filtered. 10  $cm^3$  of said solution was mixed with 10  $cm^3$  of an 8% gelatine solution. The gelatine used was previously made practically chloride-free by washing it with water.

The gelatine mixture was then mixed in the dark, while stirring, with 1  $cm^3$   $AgNO_3$  solution of 0.1 normal, and spread out on photographic paper treated with barytes. On 150  $cm^2$  paper about 3  $cm^3$  emulsion was used. The emulsion-carrying paper thus obtained was dried in a dark drying tunnel.

The dry paper was exposed in diffuse daylight. After about 20 minutes already a shade of color was seen. The exposure was continued for about 1½ hours and the exposed paper was then treated for about 5 minutes in a one per thousand solution of  $KCN$  in water, whereupon it was washed with fresh water for about half an hour and then dried. A red picture was thus obtained.

*Example 3*

A light-sensitive paper with the silver salt of 2,2'-dinitro-benzidine-dioxamic acid was produced in the manner described in Example 2, and thereafter exposed and treated in the same way. A yellow-colored picture was obtained.

*Example 4*

A light-sensitive paper with the silver salt of  $\alpha$ -nitro-oxanilic acid was produced in the manner described in Example 2, and after exposure

75

was treated in the same way. An orange-colored picture was obtained.

*Example 5*

5 A light-sensitive paper with the silver salt of p-nitro-oxanilic acid was produced and treated as in Example 4. A yellow picture was obtained after exposure.

*Example 6*

10 A light-sensitive paper with the NH<sub>4</sub>-salt of 2,2'-dinitro-benzidine-di-oxamic acid was produced in the same way as the silver salt in Example 3. After exposure the exposed material was only washed with water, whereby the unexposed part was washed out. A yellow-colored picture was obtained.

15 While I have described my invention in a detailed and comprehensive manner and provided specific examples of executing the same, it is to 20 be understood that no limitations are intended other than those imposed by the scope of the claims.

I claim as my invention:

1. A light-sensitive photographic layer suitable 25 for the production of colored images containing a light-sensitive salt of a substituted oxalic acid in which a carboxyl group has been coupled with an amino group of an organic dye, which salt upon exposure and such development as may be desirable is separable into a relatively soluble cation-containing fragment removable by solution, as is the unexposed salt, and a relatively insoluble organic fragment which remains to yield a colored image.

35 2. A light-sensitive photographic layer suitable for the production of colored images containing a light-sensitive metal salt of a substituted oxalic acid in which a carboxyl group has been coupled with an amino group of an organic dye, which salt upon exposure and such development as may be desirable is separable into a relatively soluble cation-containing fragment removable by solution, as is the unexposed salt, and a relatively insoluble organic fragment which remains to yield 40 a colored image.

45 3. A light-sensitive photographic layer suitable for the production of colored images containing a light-sensitive silver salt of a substituted polybasic acid in which a carboxyl group has been coupled with an amino group of a dye, which salt upon exposure and such development as may be desirable is separable into a relatively soluble cation-containing fragment removable by solution, as is the unexposed salt, and a relatively insoluble organic fragment which remains to yield 55 a colored image.

50 4. A light-sensitive photographic layer suitable for the production of colored images containing a light-sensitive metal salt of a substituted oxalic acid in which a carboxyl group has been coupled with an amino group of an azo dye, which salt upon exposure and such development as may be desirable is separable into a relatively soluble cation-containing fragment removable by solution, as is the unexposed salt, and a relatively insoluble organic fragment which remains to yield 60 a colored image.

65 5. A light-sensitive photographic layer suitable for the production of colored images containing a light-sensitive metal salt of a substituted oxalic acid in which a carboxyl group has been coupled with an amino group of a nitro dye, which salt upon exposure and such development as may be desirable is separable into a relatively soluble cation-containing fragment removable by solu- 70

tion, as is the unexposed salt, and a relatively insoluble organic fragment which remains to yield a colored image.

6. A light-sensitive photographic layer suitable for the production of colored images containing a light-sensitive metal salt of a substituted oxalic acid in which a carboxyl group has been coupled with an amino group of a bis-azo dye, which salt upon exposure and such development as may be desirable is separable into a relatively soluble cation-containing fragment removable by solution, as is the unexposed salt, and a relatively insoluble organic fragment, which remains to yield a colored image.

10 7. A light-sensitive photographic layer suitable for the production of colored images containing as an image and color-forming agent a light-sensitive silver salt of a substituted oxalic acid in which a carboxyl group has been coupled with an amino group of an azo dye.

15 8. A light-sensitive photographic layer suitable for the production of colored images containing as an image and color-forming agent a light-sensitive silver salt of a substituted oxalic acid in which a carboxyl group has been coupled with 20 an amino group of a nitro dye.

25 9. A light-sensitive photographic layer suitable for the production of colored images containing as an image and color-forming agent a light-sensitive silver salt of a substituted oxalic acid in which a carboxyl group has been coupled with 30 an amino group of a bis-azo dye.

35 10. A light-sensitive photographic layer suitable for the production of colored images containing as an image and color-forming agent, the com- 35



45 11. A light-sensitive photographic layer suitable for the production of colored images containing as an image and color-forming agent, the compound



55 12. A light-sensitive emulsion suitable for producing colored images by photography and containing as a light-sensitive agent a metal salt of a substituted oxalic acid in which a carboxyl group has been coupled with a polar group of a dye, which salt upon exposure and such development as may be desirable is separable into a relatively soluble cation-containing fragment removable by solution, as is the unexposed salt, and a relatively insoluble organic fragment which remains to yield a colored image.

60 13. A light-sensitive photographic layer suitable for the production of colored images containing a member selected from the group consisting of light-sensitive polycarboxylic acids and light-sensitive polycarboxylic acid metal salts in each of which a carboxyl group has been coupled with an amino group of an organic dye, which compound upon exposure and such development as may be desirable, is separable into a relatively soluble fragment removable by solution, as is the unexposed compound, and a relatively insoluble fragment which remains to yield a colored image.

65 14. A light-sensitive photographic layer suitable for the production of colored images con- 70

taining a member selected from the group consisting of light-sensitive dicarboxylic acids and light-sensitive dicarboxylic acid metal salts in each of which a carboxyl group has been coupled with an amino group of an organic dye, which compound upon exposure and such development as may be desirable is separable into a relatively soluble fragment removable by solution, as is the unexposed compound, and a relatively insoluble fragment which remains to yield a colored image.

15. A light-sensitive photographic layer suitable for the production of colored images con-

taining a member selected from the group consisting of light-sensitive oxalic acids and light-sensitive oxalic acid metal salts in each of which a carboxyl group has been coupled with an amino group of an organic dye, which compound upon exposure and such development as may be desirable is separable into a relatively soluble fragment removable by solution, as is the unexposed compound, and a relatively insoluble fragment which remains to yield a colored image. 16

HENRICUS JACOBUS CHARLES TENDELOO.